

## UNITED STATES PATENT OFFICE

WOLF KRITCHEVSKY, HAROLD C. PRUTSMAN, AND ELLIOTT MORRILL, OF CHICAGO, ILLINOIS, ASSIGNORS TO RIT PRODUCTS CORPORATION, OF CHICAGO, ILLINOIS, A CORPORATION OF DELAWARE

## DYE

No Drawing.

Application filed December 3, 1928. Serial No. 323,564.

Our invention relates to a product known as package dyes for home use, and particularly to an improvement on the dye disclosed in several prior patents, relating to a combination of dye and soap, one of which is No. 1,610,291 dated December 14, 1926.

In the production of dyes of the character mentioned, the manufacturer is confronted with the problem of preparing a product that will enable the user to produce results that will equal or approximate the results obtained by a commercial dyeing house. This problem is difficult because in the commercial dyeing establishments the work is done by experts who have at hand the proper dyes, mordants, fillers, penetrators and mechanical equipment.

Inasmuch as the individual buyer cannot be trained or educated to perform the operations in a skillful manner, the product should be so prepared that it will be, in effect, "fool-proof"; in other words, a product that will except under unusual or abnormal conditions insure satisfactory results. Such a dye should contain proper dyes in correct proportion and mixture, together with the necessary dye assistants such as mordants, fillers, diluents and penetrators.

We have found that when a product is made which consists of the proper dyes, the necessary fillers or mordants, such as common salt, Glauber's salt or starch; the necessary diluents and solvents such as water and alcohol, together with a percentage of alkylated naphthalene sulphonic acid or its salts, or in general a sulphonic acid salt of an alkylated polynuclear hydrocarbon, the product is eminently satisfactory for home use. It results in a preparation having a high degree of solubility, excellent penetrating effect, evenness of shade and softness of fabric, and enables home dyeing with practically perfect results.

Referring to the alkylated polynuclear hydrocarbons, and especially to the alkylated naphthalene sulphonic acids, their use is especially recommended on account of their high wetting power.

These compounds were developed in the after-war period in Germany to act as a sub-

stitute for soap, but they not only substitute for soap but are useful in reducing the surface tension of liquids, and increase penetration. The manufacture of some of these compounds is described in the German Patent No. 336,558, one of which especially described consisting in treating naphthalene with sulphuric acid and afterwards condensing it with iso-propyl-alcohol. A little different method is described in English Patent No. 302,258 and quite a number of different products are described.

They all consist in sulphonating naphthalene or a polynuclear hydrocarbon of the aromatic or hydro-aromatic series and then condensing them with an aliphatic, aromatic-aliphatic and hydro-aromatic alcohol, or in general, a compound containing an alcohol group. It is essential that the alcohol has at least three carbon atoms, methyl alcohol or ethyl alcohol will not give it the wetting properties. On the other hand, iso-propyl alcohol or butyl alcohols, or butylene glycol are eminently satisfactory. Also, ethylene glycol-monopropyl ether can be used. Also cyclo-hexanol, benzylalcohol, and the like. The side chains may also link together two aromatic nuclei as is the case, for instance, in the condensation products of formaldehyde with naphthalene sulphonic acids, as expressed in the U. S. Patent No. 1,722,904. The said sulphonic acids may also contain other substituents such as halogen atoms or nitro or amine or hydroxyl groups and the side chain may also be attached to such substituents as for example in amyl-naphthylamine sulphonic acids may be employed in the state of free acids or of salts.

The actual chemical composition of these compounds is not known exactly; Dr. A. Laundolt in Melland, vol. 9, page 759 describes the condensation product of sulphonated naphthalene with iso-propyl alcohol with the following graphic formula:



85

100

On the other hand, in the book by Curtis, "Die Pigment Farbstoffen" page 16, the formula is given:



10 For this reason we shall refer to those compounds merely as alkylated polynuclear hydrocarbons, which will designate them more or less properly.

15 The above mentioned compounds are sold on the market under the commercial names of Nekal products by the I. G. Neomorpine, by the Newport Chemical Co.; Terisol by the Chemical and Dye Corporation.

20 The characteristic group of those compounds is the hydrocarbon residue linked with an alkyl group and a sulphonic acid group.

25 Compounds prepared in this way give the public a very convenient, and especially technically perfect way of dyeing materials which they themselves could never achieve without knowing the properties of different wetting materials as related to the dyes, and 30 without knowing the proper proportions in order to obtain the best results.

35 By using our composition of matter in which we select the right type of dye and combine it with the right type of wetting agent, a composition of matter is obtained that can be used by any layman directly, without any technical knowledge whatsoever by simply placing the composition of matter into the proper solvent or suspending agent, like water, then treating the desired article in it by immersion, and, if necessary, heating for a length of time required until the proper shade of color is obtained, then taking it out, drying and pressing it.

40 The composition of matter can be produced either in solid form, such as cakes that are easily soluble in water, or in the form of a paste, or liquid in solution, depending upon the nature of the market and the nature of the product to be dyed.

45 A few examples of combinations that will give the desired result are as follows:

50 1. 21% direct black, C. I. 581, 10% iso-propyl naphthalene sodium sulphonate, 69% common salt.

55 2. 1% of alkali blue, C. I. 704, 2% of iso-propylated naphthalene potassium sulphonate, 97% Glauber's salt.

60 3. 5% of cyanone blue, 5R, C. I. 289, 5% direct blue BB, C. I. 406, 8% of iso-propylated naphthalene ammonium sulphonate, 2% sulphonated soap, 80% common salt.

65 4. 1% of acid violet, 3B, C. I. 698, 1% of iso-propyl naphthalene sodium sulphonate, 97% water, 1% soap.

5. 3% methylene blue, C. I. 922, 1% of butylated naphthalene ammonium sulphonate, 25% alcohol, 71% water.

6. 6% methylene blue, C. I. 922, 12% butylated naphthalene ammonium sulphonate, 70% gum arabic, 50% water.

7. 50% rhodamine B, C. I. 749, 50% amy- lated naphthalene potassium sulphonate.

8. 33% alizarine blue, C. I. 1054, 15% iso-propylated naphthalene sodium sulphonate, 15% sulphonated soap, 10% ammonium sulphate, 27% common salt.

9. 2% eosine, C. I. 768, 2% iso-propyl naphthalene sulphonic acid, 48% alcohol, 48% water.

In these examples, we have shown a few of many possible variations. The different chemicals and dyes can be interchanged, their quantities varied, the product substituted by equivalents, and the finished product may be in liquid, solid or paste form.

Instead of dyes mentioned above, any other dyes of commerce or mixtures thereof, that will furnish the results required can be substituted. Instead of ordinary salts like Glauber's salts, other salts like chromium or chromate salt can be used.

We claim:

1. A composition of matter adapted to be dispensed in packages and to be combined with a liquid for use, comprising sulphonic acid salt of an alkylated polynuclear hydrocarbon residue possessing a high wetting power, and a water soluble dye.

2. A composition of matter adapted to be dispensed in packages and to be combined with a liquid for use, comprising a water soluble dye and a sulphonate acid salt of a substituted polynuclear aromatic hydrocarbon possessing high wetting power.

3. A composition of matter adapted to be dispensed in packages and to be combined with a liquid for use, comprising a water soluble dye and a chemical possessing a high wetting power of the general composition



in which Y indicates the hydrocarbon residue, X designates hydrogen, any metal like potassium, sodium, ammonium and its substitution products, and R designates an alkyl group containing not less than three carbon atoms, like isopropyl, butyl or benzyl.

4. A composition of matter adapted to be dispensed in packages and to be combined with a liquid for use, comprising a water soluble dye and an alkylated derivative of a salt of naphthalene sulphonate acid possessing high wetting properties.

5. A composition of matter adapted to be dispensed in packages and to be combined with a liquid for use, comprising a water sol-

uble dye and a salt of iso-propyl naphthalene sulphonic acid.

6. A composition of matter adapted to be dispensed in packages and to be combined with a liquid for use, comprising a water soluble dye and a salt of iso-propyl naphthalene sulphonic acid, and a dye assistant.

7. A composition of matter adapted to be dispensed in packages and to be combined with a liquid for use, comprising a water soluble dye and a chemical possessing a high wetting power of the general composition



15 in which Y indicates the hydrocarbon residue, X designates hydrogen, any metal like potassium, sodium, ammonium and its substitution products, and R designates an alkyl group containing not less than three carbon atoms, like isopropyl, butyl or benzyl, and a dye assistant.

In testimony whereof we have affixed our signatures.

25 W. KRITCHEVSKY.  
H. C. PRUTSMAN.  
ELLIOTT MORRIEL.

30

35

40

45

50

55

60

65